# EUROPEAN PATENT SPECIFICATION

(11) **EP 2 513 408 B1**
(45) Date of publication and mention of the grant of the patent: **18.06.2014**
(21) Application number: 10790969.9
(22) Date of filing: 14.12.2010
(51) Int. Cl.: E21B 17/00, E21B 43/12, E21B 17/01, E21B 17/08

(54) **INHIBITING LIQUID LOADING, CORROSION AND/OR SCALING IN OILFIELD TUBULARS**
VERHINDERUNG VON FLÜSSIGKEITSBELADUNG, KORROSION UND/ODER KESSELSTEINABLAGERUNG BEI ÖLFELDROHREN
TRAITEMENT POUR EMPÊCHER LE CHARGEMENT DE LIQUIDE, LA CORROSION ET/OU L'ENTARTRAGE DANS DES ÉLÉMENTS TUBULAIRES DE CHAMP PÉTROLIFÈRE

(30) Priority: 14.12.2009 EP 09179115
(43) Date of publication of application: 24.10.2012
(73) Proprietor: Shell Internationale Research Maatschappij B.V., 2596 HR The Hague (NL)
(72) Inventor: VEEKEN, Cornelis, Adrianus, Maria, NL-9405 TA Assen (NL)
(86) International application number: PCT/EP2010/069658
(87) International publication number: WO 2011/073204

(56) References cited:
- EP-A1- 0 608 081
- US-A- 3 878 312
- US-A- 5 209 946
- US-A1- 2009 200 013

## Description

### BACKGROUND OF THE INVENTION

The invention relates to a method for inhibiting liquid loading, corrosion and scaling in oilfield tubulars, in particular in production tubings in natural gas production wells.

Condensation of liquids in natural gas production wells may inhibit production of natural gas through such wells when the gas velocity becomes insufficient to carry these liquids to surface, a phenomenon also known as liquid loading. Condensation of liquids is triggered in almost all gas wells by expansion of the gas within the well and by the lowering of the temperature of the earth crust along the length of the wellbore from the inflow region to the wellhead. In addition, free liquid may be entering the inflow region together with the gas.

Besides triggering liquid loading, the condensed and free liquid also interacts with the tubing inner surface where, depending on the composition of liquid and tubing, it can cause unacceptable corrosion and scaling.

It is known to inhibit liquid loading of gas wells from US 2009/200013 or SPE papers 71554 and 84136.

SPE paper 71554 "Design of tubing collar inserts for producing gas wells below their critical velocity" was presented by S.A.Pura et al at the 2001 SPE Annual Technical Conference and Exhibition held at New Orleans, Louisiana, USA from 30 September to 3 October 2001.

SPE paper 85136 " Investigation of new tool to unload liquids from stripper-gas wells" was presented by A.J.Ali et al at the SPE Annual Technical Conference and Exhibition held in Denver, Colorado, USA from 5 to 8 October 2003.

SPE paper 71554 discloses that the use of open or slotted disks inserted at selected points along the length of production tubing inhibits liquid loading.

SPE paper 84136 discloses the use of a vortex device, which alters the flow structure in the production tubing and improves liquid flow.

A disadvantage of the methods known from these SPE papers is that the vortex device and open or slotted disk provide flow restrictions, which reduce the production of gas and only provide local reduction of liquid loading in the vicinity of the vortex device or open or slotted disk.

The article " Experimental Study of gas-liquid two phase-flow affected by wall surface wettability" published by T.Takamasa et al in the International Journal of Heat and Fluid Flow 29(2008) 1593-1602, Journal Homepage : www.elsevier.com/locate/ijff, describes experiments to evaluate the effect of wall surface wettability on the characteristics of upward gas-liquid two phase flow in vertical pipes. The experiments are of an academic nature and no practical implications are disclosed in this article.

There is a need to alleviate the disadvantages of the methods known from the above SPE papers and to provide a method for inhibiting liquid loading in oilfield tubular, such as production tubings in gas wells, wherein liquid loading may be inhibited along at least a substantial part of the length of a gas well and wherein there is no need to inhibit the flux of natural gas by vortex tools, open or slotted disk inserts or other flow obstructing devices.

There is also a need to inhibit contact between the tubing wall and the condensed or free liquid and to thereby inhibit corrosion and scaling of the inner surface of gas well production tubings and other oilfield tubulars.

### SUMMARY OF THE INVENTION

In accordance with the invention there is provided a method for inhibiting liquid loading, corrosion and/or scaling in an oilfield tubular by treating the inner surface of the tubular with a hydrophobic coating or lining to inhibit the formation of a liquid film contacting the surface, thereby promoting the transport of liquid as droplets flowing in an upward direction alongside said inner surface while minimizing contact between the liquid and the inner surface.

The treatment preferably comprises coating at least part of the inner surface of the oilfield tubular with a compound having a low surface energy and a low contact angle hysteresis, such as a hydrophobic coating or lining.

In accordance with the invention there is furthermore provided an oilfield tubular, of which the inner surface is treated to inhibit the creation of a liquid film and to promote the transport of liquid as droplets while minimizing contact with said inner surface.

The oilfield tubular may be a production tubing for use in a gas well of which the inner surface is provided a ceramic or fluor based hydrophobic coating, such as a fluoridated hydrocarbon coating comprising polymerized acrylic compounds.

These and other features, embodiments and advantages of the method and oilfield tubular according to the invention are described in the accompanying claims, abstract and the following detailed description of non-limiting embodiments depicted in the accompanying drawings, in which description reference numerals are used which refer to corresponding reference numerals that are depicted in the drawings.

### BRIEF DESCRIPTION OF THE DRAWINGS

Fig.1 shows a schematic of the concurrent flow of gas and liquid in a section of a gas well where the gas flow is sufficient to move both liquid film and liquid droplets upward; and
Fig.2 shows a schematic of the concurrent flow of gas and liquid in a section of a gas well where the gas flow is insufficient to move the liquid film upward but still sufficient to move the liquid droplets upward

### DETAILED DESCRIPTION OF THE DEPICTED EMBODIMENTS

Fig.1 shows a gas well 1 with liquid film 2 alongside the inner surface of the production tubing 4 and liquid droplets 3 that are dragged upward through the interior of the production tubing 4 by the upward velocity U_{gas1} of natural gas. In the situation shown in Fig.1 the upward gas velocity U_{gas1} is sufficient to also drag the liquid film 2 in an upward direction alongside the inner surface of the production tubing 4 as illustrated by the arrow U_{film↑}. Drag forces exerted by the upward gas flux will also initiate waves at the inner surface of the liquid film 2 that move in an upward direction as illustrated by arrow U_{wave↑} and with wave crests that tilt in an upward direction.

Fig.2 shows a gas well 20 with liquid film 21 and liquid droplets 22, wherein the upward gas velocity U_{gas2} is lower than the U_{gas1} shown in Fig.1.

The reduced gas velocity U_{gas2} is still sufficient to drag liquid droplets upwards but insufficient to move the liquid film 21 in an upward direction along the inner surface of the production tubing 24.

The drag forces exerted by the upward gas flux initiate waves at the inner surface of the liquid film 21, which still move upward, but at a lower speed than shown in Fig.1 and with wave crests that tilt in downstream direction. The downward velocity of the liquids in the liquid film U_{film↓} may result in liquid accumulation at the bottom of the the production tubing 24, which may inhibit and eventually terminate the influx of gas into the well 20.

Experiments have shown that applying hydrophobic coating to the inner surface of the production tubing will inhibit creation of the liquid film and will reduce the gas velocity at which liquid loading occurs by about 50%. This observation matches the upward gas velocity required to transport liquid droplets in upward direction. Liquid loading in gas wells will result in liquid accumulation at the bottom of the well, which will inhibit gas production from this well.

Inhibiting the creation of a liquid film will also inhibit corrosion and scaling at the tubing inner wall. Corrosion and scaling trigger costly preventative or corrective maintenance to either prevent or repair the detrimental effects of corrosion and scaling. Therefore, hydrophobic coating of production tubing will extend the life a wet gas production well.

Suitable hydrophobic coating materials are ceramic or fluor based coatings, such as a fluoridated hydrocarbon coating comprising polymerized acrylic compounds.

The hydrophobic coatings according to the invention may also be used to inhibit liquid loading, corrosion and/or scaling in other oilfield tubulars than production tubings in gas wells, such as in surface flowlines and/or risers for transporting natural gas, condensate and/or a multiphase mixture of crude oil, condensate and natural gas from multiphase hydrocarbon fluid production wells to hydrocarbon processing facilities.

## Claims

1. A method for inhibiting liquid loading, corrosion and/or scaling in an oilfield tubular, the method comprising treating at least part of an inner surface of the tubular to inhibit the creation of a liquid film and to promote the transport of -liquid as droplets while minimizing contact with said inner surface,
wherein the treatment comprises providing at least part of the inner surface of the oilfield tubular with a hydrophobic coating or lining,
wherein the hydrophobic coating is a ceramic or fluor based hydrophobic coating,
**characterized in that** the hydrophobic coating is a fluoridated hydrocarbon coating comprising polymerized acrylic compounds.

2. The method of claim 1, wherein the treatment comprises coating at least part of the inner surface with a compound having a low surface energy and a low contact angle hysteresis.

3. The method of claims,l or 2, wherein the oilfield tubular is a production tubing in a natural gas production well.

4. The method of claim 3, wherein the natural gas production well is a wet and/or sour natural gas production well.

5. An oilfield tubular of which the inner surface is treated to inhibit corrosion, scaling and the creation of a liquid film and to promote the transport of liquid as droplets while minimizing contact with said inner surface,
wherein the inner surface is provided with a hydrophobic coating or lining,
wherein the hydrophobic coating is a ceramic or fluor based hydrophobic coating,
**characterized in that** the hydrophobic coating is a fluoridated hydrocarbon coating comprising polymerized acrylic compounds.

6. The oilfield tubular of claim 5, wherein the treatment comprises a coating that covers at least part of the inner surface, which coating comprises a compound having a low surface energy and a low contact angle hysteresis.

7. The oilfield tubular of claims 5 or 6, wherein the oilfield tubular is a production tubing for use in a crude oil and/or natural gas production well.

8. The oilfield tubular of claim 7, wherein the oilfield tubular is a production tubing for use in a wet and/or sour natural gas production well.

9. The oilfield tubular of claim 5, wherein the oilfield tubular is a surface flowline or riser for transporting natural gas, condensate and/or a multiphase mixture of crude oil, condensate and natural gas from a multiphase hydrocarbon fluid production well to hydrocarbon processing facilities.

## Patentansprüche

1. Verfahren zur Verhinderung von Flüssigkeitsbeladung, Korrosion und/oder Kesselsteinablagerung bei einem Ölfeldrohr, wobei das Verfahren das Behandeln von mindestens einem Teil der inneren Oberfläche des Rohres zur Verhinderung der Ausbildung eines Flüssigkeitsfilmes und zur Förderung des Transports der Flüssigkeit als Tröpfchen umfasst, während der Kontakt mit der inneren Oberfläche minimiert wird,
wobei die Behandlung die Bereitstellung von mindestens einem Teil der inneren Oberfläche des Ölfeldrohres mit einer hydrophoben Beschichtung oder Auskleidung umfasst,
wobei die hydrophobe Beschichtung eine auf Keramik oder Fluor basierende hydrophobe Beschichtung ist,
**dadurch gekennzeichnet, dass** die hydrophobe Beschichtung eine fluoridierte Kohlenwasserstoffbeschichtung ist, welche polymerisierte Acrylverbindungen umfasst.

2. Verfahren nach Anspruch 1, wobei die Behandlung die Beschichtung von mindestens einem Teil der inneren Oberfläche mit einer Verbindung mit einer niedrigen Oberflächenenergie und einer niedrigen Kontaktwinkelhysterese umfasst.

3. Verfahren nach Anspruch 1 oder 2, wobei das Ölfeldrohr ein Förderrohr in einer Erdgasförderbohrung ist.

4. Verfahren nach Anspruch 3, wobei die Erdgasförderbohrung ein Naß- und/oder eine Sauergasförderbohrung ist.

5. Ölfeldrohr, von welchem die innere Oberfläche zur Verhinderung von Korrosion, Kesselsteinablagerung und zur Ausbildung eines Flüssigkeitsfilms und zur Förderung des Transports von Flüssigkeit als Tröpfchen behandelt ist, während der Kontakt mit der inneren Oberfläche minimiert wird,
wobei die innere Oberfläche mit einer hydrophoben Beschichtung oder Auskleidung versehen ist,
wobei die hydrophobe Beschichtung eine auf Keramik oder Fluor basierende hydrophobe Beschichtung ist,
**dadurch gekennzeichnet, dass** die hydrophobe Beschichtung eine fluoridierte Kohlenwasserstoffbeschichtung ist, welche polymerisierte Acrylverbindungen umfasst.

6. Ölfeldrohr nach Anspruch 5, wobei die Behandlung eine Beschichtung umfasst, welche mindestens einen Teil der inneren Oberfläche bedeckt, welche Beschichtung eine Verbindung mit einer niedrigen Oberflächenenergie und einer niedrigen Kontaktwinkelhysterese umfasst.

7. Ölfeldrohr nach Anspruch 5 oder 6, wobei das Ölfeldrohr ein Förderrohr zur Verwendung in einer Rohöl- und/oder Erdgasförderbohrung ist.

8. Ölfeldrohr nach Anspruch 7, wobei das Ölfeldrohr ein Förderrohr zur Verwendung in einer Naß- und/oder einer Sauergasförderbohrung ist.

9. Ölfeldrohr nach Anspruch 5, wobei das Ölfeldrohr eine Oberflächenfließleitung oder ein Steigrohr zum Transport von Erdgas, Kondensat und/oder einer Mehrphasenmischung aus Rohöl, Kondensat und Erdgas von einer Mehrphasenkohlenwasserstofffluid-Förderbohrung zu Verarbeitungsanlagen für Kohlenwasserstoff ist.

## Revendications

1. Méthode pour inhiber le bourrage de liquide, la corrosion et/ou l'entartrage dans un tubulaire de champ de pétrole, la méthode comprenant le traitement d'au moins une partie d'une surface intérieure du tubulaire pour inhiber la création d'un film liquide et pour promouvoir le transport de liquide comme gouttelettes tout en minimisant le contact avec ladite surface intérieure, dans laquelle le traitement comprend le fait de prévoir au moins une partie de la surface intérieure du tubulaire de champ de pétrole avec une couche ou un revêtement hydrophobique, dans laquelle la couche hydrophobique est une céramique ou une couche hydrophobique à base de fluor, **caractérisée en ce que** la couche hydrophobique est une couche d'hydrocarbure fluoré comprenant des composés acryliques polymérisés.

2. Méthode selon la revendication 1, dans laquelle le traitement comprend le revêtement d'au moins une partie de la surface intérieure avec un composé ayant une basse énergie de surface et une basse hystérésis d'angle de contact.

3. Méthode selon l'une des revendications 1 ou 2, dans laquelle le tubulaire de champ de pétrole est un tube de production dans un puits de production de gaz naturel.

4. Méthode selon la revendication 3, dans laquelle le puits de production de gaz naturel est un puits de production de gaz naturel humide et/ou acide.

5. Tubulaire de champ de pétrole duquel une surface intérieure est traitée pour inhiber la corrosion, l'entartrage et la création de film liquide et pour promouvoir le transport de liquide comme gouttelettes tout en minimisant le contact avec ladite surface intérieure, dans laquelle le traitement comprend le fait de prévoir au moins une partie de la surface intérieure du tubulaire de champ de pétrole avec une couche ou un revêtement hydrophobique, dans laquelle la couche hydrophobique est une céramique ou une couche hydrophobique à base de fluor, **caractérisée en ce que** la couche hydrophobique est une couche d'hydrocarbure fluoré comprenant des composés acryliques polymérisés.

6. Tubulaire de champ de pétrole selon la revendication 5, dans lequel le traitement comprend le revêtement d'au moins une partie de la surface intérieure avec un composé ayant une basse énergie de surface et une basse hystérésis d'angle de contact.

7. Tubulaire de champ de pétrole selon l'une des revendications 5 ou 6, dans lequel le tubulaire de champ de pétrole est un tube de production pour l'usage dans un puits de production de pétrole brut et/ou de gaz naturel.

8. Tubulaire de champ de pétrole selon la revendication 7, dans lequel le tubulaire de champ de pétrole est un tube de production pour l'usage dans un puits de production de gaz naturel humide et/ou acide.

9. Tubulaire de champ de pétrole selon la revendication 5, dans lequel le tubulaire de champ de pétrole est une conduite d'écoulement en surface ou une colonne montante pour transporter du gaz naturel, du condensat et/ou un mélange polyphasique de pétrole brut, de condensat et de gaz naturel d'un puits de production de fluide hydrocarbure polyphasique vers des installations de traitement.
